

# United States Patent [19]

Willems et al.

[11] 3,841,877

[45] Oct. 15, 1974

[54] **DEVELOPMENT OF EXPOSED  
PHOTOGRAPHIC SILVER HALIDE  
ELEMENTS**

[75] Inventors: **Josef Frans Willems, Wilrijk;  
Antoon Leon Vandenberghe, Hove;  
Robert Joseph Pollet, Vremde;  
Raymond Albert Roosen, Gravenweze;  
Herman Adelbert Philippaerts, Edegem, all of Belgium**

[73] Assignee: **Agfa-Gevaert N.V., Mortsel, Belgium**

[22] Filed: **Nov. 3, 1972**

[21] Appl. No.: **303,406**

[30] **Foreign Application Priority Data**

Nov. 10, 1971 Great Britain ..... 52288/71

[52] U.S. Cl. ..... **96/56, 96/55, 96/59,  
96/66.3, 96/76 R, 96/95**

[51] Int. Cl. ..... **G03c 7/00, G03c 5/50, G03c 1/06**

[58] **Field of Search ..... 96/66, 22, 55, 56, 59,  
96/76, 95**

[56] **References Cited**

UNITED STATES PATENTS

3,246,988 4/1966 Porter ..... 96/66 R

|           |         |                     |            |
|-----------|---------|---------------------|------------|
| 3,295,978 | 1/1967  | Barr .....          | 96/95      |
| 3,379,529 | 4/1968  | Porter .....        | 96/66 R    |
| 3,493,539 | 2/1970  | Skoutchi .....      | 119/155 UA |
| 3,615,522 | 10/1971 | Ohi .....           | 96/66 R    |
| 3,756,821 | 9/1973  | Hayashi et al. .... | 96/66 R    |

*Primary Examiner—Mary F. Kelley  
Attorney, Agent, or Firm—A. W. Breiner*

[57] **ABSTRACT**

A method is described of developing an exposed photographic silver halide material in an alkaline medium in the presence of a 2,3— or 2,5—dihydroxyphenylbenzotriazole. Upon development, development inhibiting benzotriazole compounds are released at the site of exposure. The method is particularly suitable for the development of photographic colour elements to reduce the contrast and for the development of emulsions of the Lippmann-type to reduce distortions of closely adjacent image details, to promote image-sharpness and to reduce yellow staining upon reversal processing.

**17 Claims, No Drawings**

# DEVELOPMENT OF EXPOSED PHOTOGRAPHIC SILVER HALIDE ELEMENTS

The present invention relates to developing agents for silver halide emulsions, which upon development release benzotriazole development-inhibiting compounds.

It is known from British Pat. Specification 1,058,606 filed Feb. 27, 1964 by Eastman Kodak Co. to employ in silver halide photography hydroquinone derivatives, which by activation with an alkaline medium develop the exposed silver halide and release development-inhibiting 1-substituted tetrazolylthiols at or near the site of exposure, which results in reduced contrast with little or no loss of speed and enhanced sharpness. In the development of the latent image these hydroquinone derivatives may be used either as the sole developing agent or in conjunction with another developing agent.

In accordance with the present invention it was found that 2,3-dihydroxyphenylbenzotriazoles and 2,5-dihydroxyphenylbenzotriazoles, which are known in the literature as U.V.-absorbing compounds, see e.g. U.S. Pat No. 3,493,539 of Martin Skoultchi, Joseph Fertig and Leonard I. Nass issued Feb. 3, 1970 are suitable for the same purpose as the above hydroquinone derivatives in that, when used in alkaline medium, they release at the site of exposure benzotriazole compounds, which slow down development.

The dihydroxyphenyl nucleus may be further substituted and carry any of the known substituents used in hydroquinone and pyrocatechol type developers, e.g. alkyl, aryl, halogen, hydroxyl, alkoxy, etc. The benzotriazole group may also carry further substituents e.g. halogen, alkyl, nitro, amino, sulpho, acylamino, etc. and may carry a fused-on benzene nucleus. Further, the dihydroxyphenyl group may be linked either to the 1-position or the 2-position of the benzotriazole.

The 2,3- or 2,5-dihydroxyphenylbenzotriazoles may also be used in a chemically masked form, particularly when added to the photographic material, as is known to be done for dihydroxybenzene developing agents (cfr. U.S. Pat. No. 3,246,988 of Ralph F. Porter and Thomas E. Gompf issued Apr. 19, 1966 and Belgian Pat. No. 734,140 filed June 6, 1969 by Gevaert-Agfa N.V.) e.g. in the form of derivatives of these dihydroxyphenylbenzotriazoles in which at least one of the hydroxyl groups has been esterified to form a hydrolyzable acyloxy, halocycloxy or acyloxy group with quaternary ammonium substituent.

Thus, the present invention provides a method of producing a photographic image, which comprises developing an exposed photographic material comprising a support and a silver halide emulsion layer in an alkaline medium in the presence of a 2,3- or 2,5-dihydroxyphenylbenzotriazole compound.

Though the 2,3- or 2,5-dihydroxyphenylbenzotriazole compound may be used in a photographic silver halide developing composition as the sole developing agent, it is preferable to use the said compound in the presence of another developing agent, which may be a black-and-white developing agent e.g. hydroquinone or a colour developing agent, e.g. an aromatic primary amino colour developing agent.

In accordance with the present invention it is preferred to employ the 2,3- or 2,5-dihydroxyphenylbenzotriazole compound or its chemically masked form

as described above in the photographic material having a silver halide emulsion layer, either in the emulsion layer or in a water-permeable layer adjacent thereto, and to carry out development when the emulsion layer has been exposed, by treating the material with a conventional black-and-white or colour developing composition.

The concentration of the compounds of the invention in the emulsion is dependent on the characteristics of the emulsion and is therefore best determined by trial. In most cases, the optimum concentration in the emulsion is between about 50 mg and 5 g, preferably between about 200 mg and 2 g per mole of silver halide.

Photographic silver halide emulsions useful in the present invention comprise any of the ordinarily employed silver halide emulsions e.g. silver chloride, silver chlorobromide, silver chlorobromoiodide, silver bromide, and silver bromoiodide emulsions. Any of the conventionally employed water-permeable hydrophilic colloids can be employed in the silver halide emulsions and the other water-permeable layers contiguous thereto. Typical water-permeable colloids include gelatin, albumin, polyvinyl alcohols, agar agar, sodium alginate, hydrolysed cellulose esters, hydrophilic polyvinyl copolymers, etc.

The emulsions may be coated on a wide variety of photographic emulsion supports. Typical supports include cellulose ester film, polyvinyl acetal film, polystyrene film, polyethylene terephthalate film and related films of resinous materials as well as paper and glass.

The light-sensitive emulsions to which the development inhibitor releasing compounds of the invention are added may be sensitized chemically as well as spectrally.

The emulsions may be sensitized chemically by any of the accepted procedures. They may be digested with naturally active gelatin or in the presence of small amounts of sulphur-containing compounds such as allyl thiocyanate, allyl thiourea, sodium thiosulphate, etc. The emulsions may also be sensitized by means of reducers, e.g. tin compounds as described in British Pat. No. 789,823 filed Apr. 29, 1955 by Gevaert Photo-Producten N.V., polyamines e.g. diethyltriamine, and small amounts of noble metal compounds such as gold, platinum, palladium, iridium, ruthenium and rhodium as described by R. Koslowsky, Z. Wiss. Phot. 46, 67-72 (1951). Of course, the emulsions may also be sensitized chemically by the combined use of these chemical sensitizers.

Emulsions stabilizers or antifoggants may be added to the silver halide emulsion e.g. aliphatic, aromatic and heterocyclic mercapto compounds preferably comprising sulpho groups or carboxyl groups, mercury compounds as those described in Belgian Pat. No. 524,121 filed Nov. 7, 1953 by Kodak Ltd., Belgian Pat. No. 677,337 filed Mar. 4, 1966 by Gevaert-Agfa N.V., Belgian Pat. No. 707,386 filed Dec. 1, 1967 by Gevaert-Agfa N.V. and Belgian Pat. No. 709,195 filed Jan. 11, 1968 by Gevaert-Agfa N.V., in British Pat. No. 1,173,609 filed Dec. 12, 1966 by Agfa-Gevaert N.V., and in U.S. Pat. No. 3,179,520 of Yoshio Miura, Akira Kumai and Yosuke Nakajima issued Apr. 20, 1965 and tetraazaindenes as described by Birr in Z. wiss. Phot. 47, 2-58 (1952) e.g. the hydroxy tetra-azaindenes such as 5-methyl-7-hydroxy-s-triazolo[1,5-a]pyrimidine.

The emulsions may further comprise the known speed-increasing alkylene oxide compounds and onium compounds. The alkylene oxide compounds include alkylene oxide condensation products or polymers as described in U.S. Pat. No. 1,970,578 of Conrad Schöller and Max Wittner issued Aug. 21, 1934, U.S. Pat. No. 2,240,472 of Donald R. Swan issued Apr. 29, 1941, U.S. Pat. No. 2,423,549 of Ralph Kingsley Blake, William Alexander Stanton and Ferdinand Schulze issued July 8, 1947, U.S. Pat. No. 2,441,389 of Ralph Kingsley Blake issued May 11, 1948, U.S. Pat. No. 2,531,832 of William Alexander Stanton issued Nov. 28, 1950 and U.S. Pat. No. 2,533,990 of Ralph Kingsley Blake issued Dec. 12, 1950 and in British Pat. No. 930,637 filed May 7, 1959 by Gevaert Photo-Producten N.V., British Pat. No. 940,051 filed Nov. 1, 1961 by Gevaert Photo-Producten N.V., British Pat. No. 945,340 filed Oct. 23, 1961 by Gevaert Photo-Producten N.V., British Pat. No. 991,608 filed June 14, 1961 by Kodak Ltd. and British Pat. No. 1,015,023 filed Dec. 24, 1962 by Gevaert Photo-Producten N.V. The onium compounds may be of the ammonium, phosphonium and sulphonium type, e.g. trialkyl sulphonium salts, tetra-alkylammonium salts, alkyl pyridinium and alkyl quinolinium salts, bisalkylene pyridinium salts, quaternary ammonium and phosphonium polyoxyalkylene salts, etc.

The compounds of the invention may be used in various kinds of photographic emulsions. In addition to being useful in X-ray and other non-optically sensitized emulsions, they may also be used in orthochromatic, panchromatic and infrared-sensitive emulsions. They may be used in emulsions intended for colour photography, e.g. emulsions containing colour forming couplers or emulsions to be developed by solutions containing couplers. They may be used in emulsions intended for use in the well-known diffusion transfer process, which utilize the undeveloped silver halide in the non-image areas of the negative to form a positive by dissolving the undeveloped silver halide and precipitating it on a receiving layer in close proximity to the original silver halide emulsion layer.

The compounds of the invention are particularly useful in emulsions intended for colour photography where during development, at the exposed areas, the oxidized aromatic primary amino colour developing agent couples with a colour forming component to form a dye image. By the presence of the compound of the invention in the emulsion, the development inhibitor is image-wise released, which results in reduced graininess and the hydroquinone developer locally regenerates the aromatic primary amino colour developing agent from its oxidation products.

The compounds of the invention were further found to be particularly suitable for use in silver halide emulsions of the Lippmann-type having an average silver halide grain-size of less than 100 nm as used e.g. for the preparation of masks in the production of microelectronic integrated circuits. These Lippmann emulsions should have a high resolving power and acutance and allow a correct reproduction of the dimensions of the image. By means of the compounds of the invention it was found possible, both on reversal and negative processing, to reduce or eliminate the distortions of image details which often arise by mutual influence of closely adjacent image details and to promote the image-sharpness. Moreover, these compounds were found to

reduce the yellow staining often encountered with reversal processing of the Lippmann-material.

In these Lippmann-emulsions the concentration of the compounds of the invention is best determined by trial. Generally, the most suitable concentration is between 20 mg and 2 g, preferably between 100 mg and 1 g per mole of silver halide.

In the production of microelectronic integrated circuits drawings are made on highly enlarged scale of the various successive masks necessary to produce one integrated circuit whereupon the drawings are reduced if necessary in successive steps, and reproduced on a photographic plate or film material forming thereby the mask ready for use. By various photographic and chemical steps (photo-etching of lacquered plates) the images of the masks thus produced are transferred to the surface on which the integrated circuit is to be made, in order to produce the required circuit elements.

In the preparation of the masks, the exposed photographic elements can be subjected to negative processing or to reversal processing.

The photographic Lippmann-materials used in electronic mask making comprise a silver halide emulsion layer, the thickness of which is generally comprised between 3 and 8 microns, and the average grain size of which is generally less than 80 nm. the ratio of silver halide to colloid binder in the Lippmann-emulsion is preferably at least 1:2 and at most 4:1.

The Lippmann-emulsions may be prepared according to methods well known in the art and described in the literature, see e.g. P. Glafkides "Photographic Chemistry," vol. 1, 1958, pages 365-368 — Mees-James "The Theory of the Photographic Process," 1966, p. 36 and National Physical Laboratory, "Notes on Applied Science" No. 20 : "Small scale preparation of Fine-Grain (Colloidal) photographic emulsions" B. H. Crawford, London, 1960. They may also be prepared according to the technique described in French Pat. No. 2,092,505 filed Mar. 25, 1971 by Agfa-Gevaert N.V.

The Lippmann-emulsions may comprise any of the silver halides referred to above but it is favoured to use silver bromide emulsions, which may have an iodide content of at most 8 mole percent.

The Lippmann-emulsions may further comprise any of the emulsion addenda referred to hereinbefore, e.g. chemical and spectral sensitizers, speed-increasing addenda of the oxyalkylene and onium type, stabilizers, and antifoggants.

The Lippmann-emulsions for microelectronic mask making are most advantageously sensitized for the green region of the spectrum. The exposure light is preferably chosen so that it has a wavelength, to which the emulsion has been spectrally sensitized.

The emulsions may further comprise light-absorbing dyes, which are chosen so that they absorb light of the wavelength, to which the material is exposed so that scattering and reflection of light within the photographic material is reduced. For more details regarding these dyes there can be referred to Belgian Pat. No. 699,375 filed June 1, 1967 by Eastman Kodak Co. and Belgian Pat. No. 742,954 filed Dec. 11, 1969 by Gevaert-Agfa N.V. The dyes are preferably used in such amounts that per micron of emulsion layer thickness a density comprised between 0.05 and 0.20, measured in the spectral region of the exposure light, is obtained.

Any of the hardening agents for hydrophilic colloids may be used in the Lippmann-emulsions comprising the compounds of invention e.g. chromijum, aluminium and zirconium salts, formaldehyde, dialdehydes, hydroxyaldehydes, acrolein, glyoxal, halogen-substituted aldehyde acids such as mucochloric and mucobromid acid, diketones such as divinyl ketone, compounds carrying one or more vinylsulphonyl groups such as divinyl sulphone, 1,3,5-trivinylsulphonyl benzene, hexahydro-s-triazines carrying vinylcarbonyl, halogenoacetyl and/or acyl groups such as 1,3,5-triacryloyl-hexahydro-1,3,5-triazine, 1,3-di-acryloyl-5-acetylhexahydro-1,3,5-triazine, 1,3,5-tri-chloroac-

ethylhexahydro-1,3,5-triazine, etc.

The Lippmann-emulsions may be coated on any of the photographic supports referred to above. In the manufacture of high resolution plate materials for the preparation of masks for use in the electronic industry, glass supports are most advantageously used in view of their high dimensional stability.

In order to promote adhesion of the Lippmann-emulsions to glass supports, the silicon compounds described in co-pending British Patent Application 54678/68 can be incorporated into the emulsion. The following examples illustrate the present invention. Example 1

The sensitometric effects of 2-(2,5-dihydroxyphenyl) benzotriazole when used in the colour development of a photographic silver halide colour material are illustrated as follows.

A photographic material comprising a film support and a silver bromoiodide emulsion (2.3 mole percent iodide), which comprises as cyan forming colour coupler the compound of the structure:



was divided into three samples.

The three samples were exposed under identical circumstances through a wedge with constant 0.30. One sample was then colour processed in the conventional way wherein development took place for 8 min. at 20° C in a developer of the following composition:

The other samples were colour processed under identical circumstances using, however, developers B and C respectively which differ from developer A only in that per litre was added 1.8 mmole of hydroquinone and 1.8 mmole of 2-(2,5-dihydroxyphenyl)benzotriazole respectively.

In the following table are given: the values obtained for the speed, gradation, maximum density, fog and percentage side-absorption of the cyan wedge image in the blue and green regions of the spectrum. The values given for the speed, gradation and maximum density are relative values; a value of 100 is given to the sample developed in developer A.

Table

| Developer | Speed | Gradation | D <sub>max</sub> | Fog  |       | % side absorption |      |
|-----------|-------|-----------|------------------|------|-------|-------------------|------|
|           |       |           |                  | blue | green | red               | blue |
| A         | 100   | 100       | 100              | 0.08 | 0.05  | 0.05              | 14   |
| B         | 66    | 43        | 67               | 0.09 | 0.05  | 0.03              | 14   |
| C         | 131   | 81        | 100              | 0.09 | 0.05  | 0.05              | 13   |
|           |       |           |                  |      |       |                   | 11   |

From the above results it appears that when using hydroquinone the reduction in gradation is accompanied with a serious loss in speed and maximum density. With 2-(2,5-dihydroxyphenyl)benzotriazole on the contrary the gradation is lowered and the speed and maximum density are not reduced.

30 The fog and percentage side-absorption remains practically unaffected.

#### Example 2

This example illustrates the use of 2-(2,5-dihydroxyphenyl)benzotriazole in Lippmann-emulsions.

A silver bromide emulsion comprising per kg 72 g of silver bromide and 93 g of gelatin was prepared by simultaneous addition of a silver nitrate solution and a potassium bromide solution to a 3 percent aqueous solution of gelatin. The conditions of precipitation were adjusted so that a Lippmann-emulsion with an average grain-size of 70 nm was obtained. Details as to the preparation of Lippmann emulsions can be found amongst others in P. Glafkides "Photographic chemistry," Vol. I, 1958, Fountain Press, London.

40 The emulsion was sensitized by addition of 150 mg per 100 g of silver halide of a merocyanine dye by means of which a strong spectral sensitization in the region of 520-550 nm was obtained. Then, an amount of the light-absorbing dye having the following structural formula:



55 was added so as to obtain, after the emulsion is coated, a density of 0.10 per micron of emulsion layer thickness, measured at 550 nm (absorption maximum of the light-absorbing dye used).

60 The emulsion was divided into 2 portions and to one of these portions 2-(2,5-dihydroxyphenyl)benzotriazole was added in an amount of 500 mg per mole of silver halide.

|                                          |      |       |
|------------------------------------------|------|-------|
| water                                    | 800  | ml    |
| N,N-diethyl-p-phenylene diamine sulphate | 2.75 | g     |
| hydroxylamine                            | 1.2  | g     |
| sodium hexametaphosphate                 | 2    | g     |
| anhydrous sodium sulphite                | 2    | g     |
| potassium carbonate                      | 75   | g     |
| potassium bromide                        | 2.5  | g     |
| water to make                            | 1    | litre |

The emulsion portions were coated on glass plates pro rata of 230 ml per sq.m so as to obtain after drying a layer thickness of 6 microns. The 2 plate materials A and B, were then exposed under identical circumstances by means of monochromatic light, the spectral composition of which corresponds with the absorption region of the light-absorbing dye used, through a test pattern, as normally used for the quantitative evaluation of materials for use in microelectronics mask-making, consisting of lines which are separated by spaces of the same width as the lines themselves and with a width varying from 1 to 20 microns. The exposure was of such an intensity so as to limit the density in the transparent areas of the images produced, which correspond with the white lines of the test pattern, to the fog value.

After the exposure the 2 plate materials were reversal processed at 20° C, under completely identical circumstances.

For that purpose the exposed materials were first developed for about 5 min. in the following developing liquid the pH of which was adjusted to 10.5:

|                                       |          |
|---------------------------------------|----------|
| hydroquinone                          | 2 g      |
| monomethyl-p-aminophenol hemisulphate | 4 g      |
| potassium bromide                     | 2 g      |
| sodium carbonate                      | 40 g     |
| sodium sulphite                       | 40 g     |
| potassium thiocyanate                 | 5 g      |
| water to make                         | 1 litre. |

The materials were then treated for about 5 min. in the following bleach bath:

|                                  |          |
|----------------------------------|----------|
| potassium dichromate             | 5 g      |
| strong sulphuric acid (d = 1.85) | 10 ccs   |
| water to make                    | 1000 ccs |

After rinsing for some minutes in water the materials were treated for 5 minutes in a clearing bath of the following composition:

|                 |          |
|-----------------|----------|
| sodium sulphite | 100 g    |
| water to make   | 1000 ccs |

After rinsing again for some minutes the materials were subjected to an overall exposure in order to render the residual silver bromide developable whereupon they were treated for about 6 minutes in the following developing liquid:

|                                       |      |     |
|---------------------------------------|------|-----|
| hydroquinone                          | 5    | g   |
| monomethyl-p-aminophenol hemisulphate | 1    | g   |
| sodium sulphite                       | 40   | g   |
| sodium carbonate                      | 30   | g   |
| potassium bromide                     | 0.5  | g   |
| water to make                         | 1000 | ccs |

Finally the materials were rinsed and dried.

From the results obtained it was clearly apparent that as compared with material B, material A to which no compound of the invention was added, showed image distortions, especially at the areas where lines of 10 to 20 microns were reproduced, and was inferior as regards yellow staining and edge sharpness.

the 2-(2,5-dihydroxyphenyl)benzotriazole used in the above examples was prepared as follows:

A solution of 24.1 g (0.1 mole) of 2-(2-hydroxy-5-methoxyphenyl)benzotriazole in 120 ml of acetic

acid and 120 ml of 48 percent hydrobromic acid was boiled for 8 hours. The precipitate formed was filtered off by suction and dissolved in 1N sodium hydroxide. The solution was decolourized with charcoal and filtered. The filtrate was acidified by means of concentrated hydrochloric acid and the precipitate formed was recrystallized from acetic acid.

Yield: 11 g (48.5 percent). Melting point: 210° C.

We claim:

1. A method of producing a photographic image, which comprises developing an image-wise exposed photographic material having a support bearing a silver halide emulsion layer, in an alkaline medium in the presence of a 2,3- or 2,5-dihydroxyphenylbenzotriazole.

2. A method according to claim 1, wherein the 2,3- or 2,5-dihydroxyphenylbenzotriazole is incorporated in a water-permeable layer on the emulsion side of the support.

3. A method according to claim 2, wherein the said water-permeable layer is a silver halide emulsion layer.

4. A method according to claim 1, wherein the alkaline medium comprises a black-and-white developing agent.

5. A method according to claim 4, wherein the said developing agent is hydroquinone.

6. A method according to claim 1, wherein the said emulsion comprises a colour forming coupler and the alkaline medium comprises an aromatic primary amino colour developing agent.

7. A method according to claim 1, wherein the said emulsion layer is a Lippmann emulsion the average grain-size of which is less than 100 nm.

8. A method according to claim 7, wherein the ratio of silver halide to hydrophilic colloid binder in the Lippmann-emulsion is comprised between 1:2 and 4:1.

9. A method according to claim 7, wherein the Lippmann emulsion is a silver bromide emulsion, which may have a silver iodide content of at most 8 mole percent.

10. A photographic material comprising a support bearing a silver halide emulsion layer, there being incorporated in a water-permeable layer on the emulsion side of the support a 2,3- or 2,5-dihydroxyphenylbenzotriazole.

11. A photographic material according to claim 10, wherein the 2,3- or 2,5-dihydroxyphenylbenzotriazole is incorporated in the said emulsion layer.

12. A photographic material according to claim 10, wherein the said emulsion layer comprises a colour forming coupler.

13. A photographic material according to claim 11, wherein the said emulsion layer is a Lippmann-emulsion layer having an average silver halide grain size of less than 100 nm.

14. A photographic material according to claim 13, wherein the ratio of silver halide to hydrophilic colloid binder in the Lippmann emulsion is comprised between 1:2 and 4:1.

15. A photographic material according to claim 13, wherein the Lippmann emulsion is a silver bromide emulsion, which may have a silver iodide content of at most 8 mole percent.

16. A photographic material according to claim 13, wherein the Lippmann-emulsion is coated on a glass support.

17. A photographic material according to claim 15, wherein the ratio of silver halide to hydrophilic colloid binder in the Lippmann emulsion is comprised between 1:2 and 4:1.

\* \* \* \* \*